

## UNITED STATES PATENT OFFICE

2,438,738

## CARROTING REAGENTS AND PROCESS

Albert Frank Bowles, Naugatuck, Conn., and Anthony J. Keegel, Jersey City, N. J., assignors to Trinity Holding Corporation, Beacon Falls, Conn., a corporation of Connecticut

No Drawing. Application February 19, 1947,  
Serial No. 729,662

3 Claims. (Cl. 8—112)

1

This application deals with the production of new and superior carotting reagents for felting animal fur fibers, particularly those of the wild rodents such as rabbits, hares, muskrats, beavers, otters, moles, and the like, and of animals of the sebraculæ species, including foxes, weasels, cats, etc. More specifically, it relates to the controlled hydrolysis and breakdown of the cystine-rich protein fibers, heretofore mentioned, so as to produce a superior felt of high quality.

In our co-pending application Serial No. 625,681, filed on October 30, 1945, now abandoned, and in our co-pending application Serial No. 630,139, filed on November 21, 1945, which is a continuation-in-part of the earlier application, and of which, this present application is a continuation-in-part, it was brought out that animal fur fibers, of the type specified above, are richer in cystine groups in the protein structure than are the fibers of other animals. It is these groups which make it possible for the fur to felt, upon treatment with the proper reagents.

It was also disclosed that, by means of the present process, there first occurs a mild hydrolysis of the amino acid-salt bridge, after which oxidation of the peptid chains takes place, resulting in the reduction of the disulfide group in the cystine portion, to form the xanthoproteic dimercaptan, resulting in a partial depolymerization or cleavage and a softening of the fiber.

According to the present invention, it has been found that a nitric acid solution of radioactive salts, particularly uranium, thorium, together with strontium, the latter metals used in the proportion to give an overall average atomic weight of 195 to 220, preferably about 200, appears to react with the dimercaptan in such a way as to produce felting properties far superior to those obtained with other carotting reagents now employed. The use of certain hydrolyzing acids, buffering salts and retarding agents aids appreciably in enhancing the felting effect. Also the use of a specific oxidizing solution, as will be subsequently described, has been found to produce a finished felt of excellent color and considerably higher tensile strength than that produced by existing methods.

In the preferred embodiment of the process of the present invention, three inorganic elements, two of which are radioactive, are employed. It is desirable to maintain at least 1% by weight of a radioactive polyvalent heavy metal of over 200 atomic weight in the concentrated carotting solution. The superiority of the radioactive elements is due not only to their inherent chemical nature,

2

but also to the fact that the radioactivity (which is of a very mild type) appears to exert a catalytic action upon the condensation reaction of the metal proteo-mercaptides in the felting operation. It has been found that a combination of uranium, thorium and strontium gives the best results, particularly when these three elements are present in proportions to give an overall average metal atomic weight of 195 to 220, and preferably about 200. Some examples of the ratios of elements which may be employed are given in the following table, although it is to be understood that other ratios are also applicable:

15

|    | Per cent U<br>(at wt. 238) | Per cent Th<br>(at wt. 232) | Per cent Sr<br>(at wt. 87.6) | Average<br>atomic<br>weight |
|----|----------------------------|-----------------------------|------------------------------|-----------------------------|
| 20 | 50                         | 25                          | 25                           | 199                         |
|    | 50                         | 30                          | 20                           | 206                         |
|    | 50                         | 27                          | 23                           | 202                         |
|    | 49                         | 27                          | 24                           | 199                         |
|    | 70                         | 5                           | 25                           | 200                         |
|    | 8                          | 70                          | 22                           | 200.7                       |

25

These elements are employed in the form of salts dissolved in nitric acid, preferably together with a small proportion of a hydrolyzing acid such as sulfuric, phosphoric or hydrochloric acids, and also preferably in presence of potassium buffering salts, such as the nitrate, sulfate, phosphate, bisulfate or bisulfite. Potassium salts are employed since they are made radioactive more readily (by presence of radioactive atoms) than buffering salts of other soluble elements.

30

A retarding agent is also employed to retard the energetic action of the mineral acid mixture.

Such an agent may be the lower fatty acids of 1-3 carbon atoms, such as formic, acetic and propionic acids, or mixtures thereof. The corresponding halo acids, such as chloracetic, fluoro-propionic, etc. may be used, provided allowance is made for the amount of halogen present (which splits off as hydrogen halide) in the amount of hydrolyzing acid used. It has been found that formic acid is not as strong a retarding agent as acetic acid, and hence it is generally employed when the fur is to be used soon. Furthermore, under the conditions existing, formic acid has a tendency to decompose, so that

40

the solution should be used within 36 hours after it is made. On the other hand, propionic acid is a stronger retarding agent than acetic acid and may be used when the fur is to be stored for some time in the wet state after carotting.

45

The oxidizing solution to be employed is gen-

erally a strong solution of hydrogen peroxide containing small amounts of hypochlorous, perchloric and chloric acids. The purpose of this solution is to remove organic nitrates produced in the ring amino acids of the peptid chains of the fur fiber, which tend to give the fur a yellowish color.

In carrying out the present invention, the following solutions are first prepared:

*Solution 1*

A 30-50% by weight of an aqueous solution of an inorganic acid of nitrogen (nitric or nitrous acid), or mixtures thereof is employed, preferably of 40-48% concentration, as for example, 46%. To this is added a small amount (0.25-0.5% by wt.), say 0.35-45%, and preferably 0.38% by weight, of a hydrolyzing acid, such as sulfuric, phosphoric, or hydrochloric acid, or mixtures thereof. A 3:1 weight ratio of  $\text{HCl}:\text{H}_2\text{SO}_4$  is preferred. There is also added 0.25-0.5% by wt. (preferably 0.38%) of a potassium buffering salt, such as potassium nitrate, and 0.2-0.5% by wt. of the retarding agent heretofore described.

The heavy polyvalent metals employed in this solution are capable of reacting with the xanthoproteic dimercaptan, and thus appear to advantageously retard the condensation reaction responsible for felting. The nitrates, sulfates, chlorides or phosphates, in the proper molal ratio to give the desired overall average atomic weight, may be employed. The acetates are toxic and are not too desirable.

The gravity of this solution is about 31.5-32° Bé.

*Solution 2*

This oxidizing solution is preferably composed of 30% aqueous hydrogen peroxide containing 5% by wt. of hypochlorous acid ( $\text{HOCl}$ ), 1% perchloric acid and 3% chloric acid. Although conventional oxidizing solutions have been found to give satisfactory results, Solution 2 has proved to give superior overall effects.

The procedure, in practicing the present invention, is to dilute Solution 1 with water to 6-14° Bé., depending on the type of pelts to be carotted. Australian pelts require 8.6-10.5° Bé., depending on the season of the year. Spring pelts require lower strength solutions than winter pelts. Summer pelts require higher concentrations. Russian skins require higher concentrations (11-14° Bé.), depending on the season of the year when the skins are taken. Domestic rabbits, such as

California whites, can be worked with gravities as low as 6° Bé.

After dilution to proper Baumé gravity, an equal volume of Solution 2 is added and the skins are treated with the resulting mixture and dried, after which they are brushed, cut, and blown, and the blown fur is then converted into hats or cloth in the conventional manner.

The invention may be more clearly understood by reference to the following examples in which are illustrated some of the many phases involved:

**EXAMPLE I**

The following solutions are prepared:

*Solution A*

|                           |      |       |
|---------------------------|------|-------|
| Water                     | lbs. | 35    |
| Potassium nitrate         | ozs. | 19.7  |
| Uranium nitrate           | ozs. | 14    |
| Thorium nitrate           | ozs. | 6     |
| Strontium nitrate         | ozs. | 4     |
| Glacial acetic acid       | ozs. | 28    |
| Hydrochloric acid (conc.) | ozs. | 28    |
| Sulfuric acid (conc.)     | ozs. | 8     |
| Nitric acid (40° Bé)      | lbs. | 101.5 |

This solution has a gravity of 32° Bé.

A lot of English coney skins was treated with the above Solution A, diluted to the strength indicated, together with Solution 2 disclosed above, in the manner heretofore outlined (i. e., as disclosed in the second and third paragraphs under "Solution 2", above. Solution A, is a specific example of "Solution 1" mentioned previously). Process F and Process B are conventional carroting methods, now employed, the tests being run under optimum conditions for each process. The following results were obtained from these tests:

Process F employs, as a carroting reagent, a solution (diluted with water to the specified gravity) of approximately the following ingredients: Water 18 lbs., nitric acid (40° Bé.) 51 lbs., sodium sulfate 4 ozs., hydrogen peroxide (100 vol.) 80 lbs., sapphire blue dye  $\frac{1}{2}$  oz. Process B employs, as a carroting reagent, a solution (diluted with water to the specified gravity) of approximately the following ingredients: Chloric acid 4 parts, perchloric acid 2 parts, nitric acid (40° Bé.) 30 parts, sulfuric acid 4 parts, hydrogen peroxide (100 vol.) 50 parts, and water 10 parts. The processing steps (except as otherwise indicated) were the same in the case of all of the methods mentioned in each series of tests.

[These tests are the result of 4 pairs the mean of which are represented by the following averages which were taken from the same brokerage lot number 134, and selected for uniformity.]

| Procedures used                         | Present invention                             | Process F                                     | Process B                                      |
|-----------------------------------------|-----------------------------------------------|-----------------------------------------------|------------------------------------------------|
| Cutter's lot number                     | 234                                           | 234                                           | 234                                            |
| Kinds of skins used                     | English coney 2d rack                         | English coney 2d rack                         | English coney 2d rack                          |
| Number of skins carrott per test        | 200                                           | 200                                           | 200                                            |
| Strength of solution                    | 6.1° Bé.                                      | 7.0° Bé.                                      | 7.0° Bé.                                       |
| Quantity of solution                    | 88 ozs.                                       | 85 ozs.                                       | 85.5 ozs.                                      |
| Color of fur after drying skins         | Natural                                       | Yellowish edges                               | Very yellow.                                   |
| Yield of fur from skins                 | 7 lb. 8 ozs.                                  | 6 lb. 15 ozs.                                 | 6 lbs. 10 ozs.                                 |
| Amt. fur blown on cone                  | 3 ozs.                                        | 3 ozs.                                        | 3 ozs.                                         |
| Size of cone used                       | 27" x 31"                                     | 27" x 31"                                     | 27" x 31"                                      |
| Hardening                               | 2 rounds 25" x 29"                            | 2 rounds 26" x 30"                            | 2 rounds 26 $\frac{1}{4}$ x 30"                |
| Starting                                | 3 rounds 21" x 27"                            | 3 rounds 23" x 29"                            | 3 rounds 23 $\frac{1}{2}$ x 29"                |
| Apron setter                            | 1 round 19.25 x 21"                           | 2 rounds 21" x 28"                            | 2 rounds 21 $\frac{1}{4}$ x 26 $\frac{1}{2}$ " |
| "A" Machine                             | 15 min. 13 x 18"                              | 19 min. 13 x 19"                              | 19 min. 13 x 19 $\frac{1}{2}$ "                |
| Boesch felter                           | 3 $\frac{1}{4}$ round 11.25 x 16.25"          | 4.5 rounds 12 x 17"                           | 5 rounds 11.5 x 17 $\frac{1}{2}$ "             |
| "B" Machine                             | 17 min. 10 $\frac{1}{2}$ x 15 $\frac{1}{4}$ " | 22 min. 10 $\frac{1}{2}$ x 15 $\frac{1}{2}$ " | 24 min. 10 $\frac{1}{2}$ x 15 $\frac{1}{4}$ "  |
| Tensile strength from 20 determinations | 52 lbs.                                       | 39 lbs.                                       | 34 lbs.                                        |
| Elongation at break                     | 68%                                           | 46%                                           | 41%                                            |
| Elastic limits                          | 26%                                           | 14%                                           | 11.5%                                          |

This grade of English coney, 2d rack, was somewhat better than the usual pelts of this grade. The fur was rather full. From the regular carroted product the yield averaged 7 lbs.

## EXAMPLE II

French white hair skins were next used with the reagents disclosed in Example I, but diluted to the strength indicated, employing the method heretofore outlined, and under comparable conditions with processes F and B to give the following test results:

[These data are the result of 3 pairs of tests, represented by the mean as given below, which were taken from brokerage lot number 352 of French white (Hare) 1st, quality selected for uniformity.]

| Procedures used                         | Present invention     | Process F                | Process B             |
|-----------------------------------------|-----------------------|--------------------------|-----------------------|
| Cutters lot number                      | 241                   | 241                      | 241                   |
| Kind of skins used                      | French white 1sts.    | French white 1sts.       | French white 1sts.    |
| Number of skins used                    | 200                   | 200                      | 200                   |
| Strength of solution                    | 8.5° Bé               | 10.5° Bé                 | 10.5° Bé              |
| Quantity of solution                    | 120 ozs.              | 132 ozs.                 | 134 ozs.              |
| Color of skin after dry                 | Slight cream          | Yellowish                | Very yellow.          |
| Condition of skins                      | Natural               | Matted                   | Matted.               |
| Yield of fur C-B                        | 9 lb. 4 oz.           | 8 lb. 10 ozs.            | 8 lb. 6 ozs.          |
| Weight blown                            | 3 ozs.                | 3 ozs.                   | 3 ozs.                |
| Size of cone 27" x 31"                  | 27" x 31"             | 27" x 31"                | 27" x 31"             |
| Hardening                               | 2 rounds 25.5 x 29.25 | 2 rounds 28 1/4 x 29 1/4 | 2 rounds 29 x 30.     |
| Starting                                | 3 rounds 20 x 26      | 3 rounds 23 x 28         | 3 rounds 23 x 29.     |
| Apron setter                            | 1 round 19 x 23       | 2 rounds 21 x 27         | 2 rounds 22 x 28.     |
| "A" Machine                             | 17 min. 14 x 19.      | 24 min. 14 x 19.         | 27 min. 14 x 19.      |
| Boesch feltier                          | 3 rounds 11 x 16      | 5 rounds 11 x 16         | 5.5 rounds 11 x 16.   |
| "B" Machine                             | 15 min. 10.5 x 15.25  | 18 min. 10.5 x 15.25     | 20 min. 10.5 x 15.25. |
| Tensile strength from 16 determinations | 69.5 lbs.             | 54.6 lbs.                | 50.2 lbs.             |
| Elongation at break                     | 63%                   | 52%                      | 46%                   |
| Elastic limits                          | 19%                   | 14%                      | 11%                   |

## EXAMPLE III

In this case, the test run was made on Australian pelts with the reagents outlined in Example I, diluted as indicated below, and in the manner already outlined, under comparable conditions for processes F and B, resulting in the following test results:

[These data are the result of 12 tests, taken from brokerage lot 619, Australian entire, selected for uniformity of fur and weight of pelts]

| Procedure used              | Present invention     | Process F                | Process B              |
|-----------------------------|-----------------------|--------------------------|------------------------|
| Lot number                  | 246                   | 246                      | 246.                   |
| Number of skins used        | 200                   | 200                      | 200.                   |
| Kind of skins used          | Australian entire     | Australian entire        | Australian entire.     |
| Strength of solution        | 9.5° Bé               | 10.5° Bé                 | 10.5° Bé.              |
| Quantity used               | 116 ozs.              | 123 ozs.                 | 125 ozs.               |
| Color after dry             | Natural               | Slight yellow            | Very yellow.           |
| Yield cut-blown             | 8 lbs. 12 ozs.        | 8 lbs. 2 ozs.            | 8 lbs.                 |
| Size of cone                | 27 x 31               | 27 x 31                  | 27 x 31.               |
| Weight formed               | 3 ozs.                | 3 ozs.                   | 3 ozs.                 |
| Hardening                   | 2 rounds 25 x 29      | 2 rounds 25 1/4 x 29 1/4 | 2 rounds 26 x 29%      |
| Starting                    | 3 rounds 21 x 27      | 3 rounds 23 1/4 x 28     | 3 rounds 23 x 28 1/4.  |
| Apron setter                | 1 1/4 rounds 19 x 21  | 2 rounds 19 x 21         | 2 1/2 round 19 x 21.   |
| "A" Machine                 | 17 min. 13 x 18       | 20 min. 13 x 18          | 20 min. 13 x 18.       |
| Boesch feltier              | 3 1/2 rounds 11 x 16  | 4 rounds 11 x 16         | 4 1/4 rounds 11 x 16.  |
| "B" Machine                 | 15 min. 10.5 x 15 1/4 | 19 min. 10.5 x 15 1/4    | 21 min. 10.5 x 15 1/4. |
| Tensile strength (16 tests) | 61 lbs.               | 44 lbs.                  | 37 lbs.                |
| Elongation at break         | 59%                   | 41%                      | 34.5%.                 |
| Elastic limits              | 21%                   | 15.4%                    | 9.6%.                  |

It will be observed that the fur obtained by employing the carotting method of the present invention has a natural to slight cream color, whereas those obtained by the other methods possessed a slight yellow to a very yellow color and had a matted appearance in some cases. Furthermore, the tensile strength of the felt made by the present invention ranged from 59 lbs. to 69.5 lbs., whereas that from the conventional methods ran 39-54.6 lbs. Also, elongation at break for felt made according to the present invention ranged 59-68%, while those made with conventional reagents ranged 34.5-52%. Elastic limits for felts made according to the present invention were 19-26%, whereas the others fell in the range 9.6-15.4%.

We claim:

1. The process of carotting fur fibers employing a medium comprising a nitric acid solution and hydrogen peroxide, the improvement comprising treating said fibers with said medium containing soluble salts of the two radioactive metals,

uranium and thorium, a soluble salt of strontium, said three salts being present in such proportion that the average atomic weight of the three metals is in the range of 195-220, a hydrolyzing agent consisting of hydrochloric and sulfuric acid and acetic acid and a soluble potassium salt.

2. In the process according to claim 1 wherein the two radioactive metal salts and soluble salt of

strontium are present in such proportion that the overall atomic weight of the three metals is about 200.

3. The process according to claim 1 in which the three polyvalent metal salts are roughly in the approximate weight proportion of uranium 21, thorium 9 and strontium 6.

4. An improved carotting reagent comprising a medium of nitric acid, hydrogen peroxide, a soluble potassium salt, a hydrolyzing mineral acid mixture comprising hydrochloric and sulfuric acids, acetic acid and a catalytic agent consisting of soluble salts of uranium, thorium and strontium, said soluble salts being present in such proportion as to have an average atomic weight of 200.

5. An improved carotting medium according to claim 4 wherein the three metal salts are present in such proportion that the overall average atomic weight of the said metal salt is between 195 and 220.

6. An improved carotting medium according to claim 4 in which the polyvalent metal salts are roughly in the weight proportion of uranium salt 7, strontium salt 2 and thorium salt 3.

7. A carotting medium according to claim 4 containing 0.25 to 0.5% by weight of a mixed hydrolyzing agent, 0.2 to 0.5% by weight of

acetic acid and 0.25 to 0.5% of a soluble potassium salt.

8. A carotting reagent for treating fur fibers comprising an aqueous solution of nitric and nitrous acids of 30-50% strength by weight; 2-4% by weight of soluble salts of uranium, thorium and strontium, said salts being present in such proportions as to have an average atomic weight of about 200; 0.25 to 0.5% by weight of hydrolyzing mineral acids mixture comprising hydrochloric and sulfuric acids; 0.2-0.5% by weight of acetic acid and 0.25-0.5% by weight of potassium nitrate.

ALBERT FRANK BOWLES.  
ANTHONY J. KEEGEL.

## UNITED STATES PATENTS

|    | Number    | Name      | Date          |
|----|-----------|-----------|---------------|
|    | 1,213,403 | Paris     | Jan. 23, 1917 |
| 5  | 1,710,565 | Bohm      | Apr. 23, 1929 |
|    | 1,955,678 | Mercier   | Apr. 17, 1934 |
|    | 2,048,645 | Fabian    | July 21, 1936 |
|    | 2,079,860 | Kauffmann | May 11, 1937  |
| 10 | 2,144,487 | Fabian    | Jan. 17, 1939 |
|    | 2,309,254 | Page      | Jan. 26, 1943 |

## FOREIGN PATENTS

|    | Number  | Country       | Date          |
|----|---------|---------------|---------------|
|    | 108,990 | Austria       | Feb. 25, 1928 |
| 15 | 471,057 | Great Britain | Aug. 20, 1937 |
|    | 631,308 | Germany       | June 17, 1936 |

## OTHER REFERENCES

Ser. No. 356,565, Haakh (A. P. C.) pub. Apr. 27, 1943.